

## UNITED STATES PATENT OFFICE

1,988,938

## COPPER ALLOY

Michael George Corson, Jackson Heights, N. Y.,  
assignor of three-twentieths to George H.  
Corey, Bayside, N. Y.

No Drawing. Application March 2, 1929, Serial  
No. 344,089. Renewed May 9, 1933

4 Claims. (Cl. 75—1)

This invention relates to alloy compositions, and particularly to the type of alloys consisting principally of copper, tin and zinc, and containing also small but effective amounts of nickel, and characterized, when treated according to the process hereinafter disclosed, by properties giving them special utility when used in forming lubricated wearing surfaces, such, for example, as in bearings, bushings, pump cylinders, gears, etc.

10 The most important feature of the copper-tin alloys (tin bronzes) that causes them to be especially suitable for use in bearings and in similar situations where resistance to wear is desirable, is their peculiar structure in the cast state, which is characterized by the presence of a soft ground mass serving as a matrix for, and containing inclusions of, a second constituent,—the beta or the delta phase,—of considerable hardness, so forming a very desirable complex possessing good bearing qualities.

15 Other alloys used for bearings, or more specifically for bushings, are certain high zinc brasses composed of a high proportion of copper in alpha phase and a low proportion in beta or in delta phase. These alloys, while they are cheaper than the high tin bronzes and can be hot worked with ease, since at high temperatures they transform into a uniform beta phase, are less satisfactory for bearing purposes than the tin bronzes, either because of insufficient hardness (too great a proportion of the softer alpha phase as compared with the harder beta phase) or because of the distribution of the harder phase in the softer ground mass in such a way as to present an excessive amount thereof at the wearing surface with consequent lack of ability to retain an adequate oil film thereon.

20 While alpha copper alloys are workable cold and to a slight extent when hot and the beta alloys are all workable hot, such alloys as are built up of mixtures of the alpha and beta phases, at any temperature below the freezing point, are not easily workable by pressure or tension either in the hot or cold state.

25 High tin bronzes are not exempt from the action of this rule. The bronzes containing between 6 and 18% tin cannot be worked while hot. Such alloys containing above 18%, and up to 27%, tin are easily workable while hot, but are relatively expensive, and, what is more important, are at room temperatures too brittle and hard throughout their structure to be useful as structural materials or for bearings and bushings.

30 I have found that ternary copper-tin-zinc bronzes can be made to behave much like com-

plex brasses in their ability to be hot worked when brought into the beta state and to retain a high strength with considerable ductility in the cold state. Also, they possess the property of high tin bronzes of being able to form a well distributed delta tin constituent of high hardness, which makes them good for wear resistance, not only because of the inherent hardness of such constituent, but also because the uniform distribution of the delta constituent in suitably sized particles throughout the ground mass or matrix imparts to a wearing surface prepared therefrom the ability to become covered with a substantial film of lubricant in the regions occupied by the softer alpha constituent of the matrix.

35 As described and claimed in my copending application Serial No. 340,651, now Patent No. 1,792,146, of which this application is in part a continuation, I have also found that such ternary bronzes can be markedly improved by structural changes resulting from a process of heat treatment. As pointed out in the aforesaid patent, such bronzes may contain additions of other elements including nickel, aluminum and manganese, which if present in controlled proportions have beneficial effects on these alloys both in their as cast condition and in their heat treated condition.

40 Alloys coming within the present invention can be prepared within the following range of proportions:

|        |                         |
|--------|-------------------------|
| Tin    | 4-18%                   |
| Zinc   | 10-35%                  |
| Nickel | Small amounts up to 10% |
| Copper | Balance                 |

45 The amounts of zinc and tin depend each upon the other. The more zinc the alloy contains, the less tin it may contain. Nickel additions within the range specified, and preferably around 2 to 3%, improve the strength and reduce the brittleness of the resulting alloy. It is found furthermore that the presence of nickel works a decided improvement in the resulting structure and accelerates the changes that take place during heat treatment. Either a part of the tin or the zinc may be replaced by about half its weight of aluminum, aluminum preferably, however, not being added in amounts greatly exceeding 2% of the total. These alloys may also contain small amounts of magnesium, phosphorus, silicon or manganese used as deoxidizers. When aluminum is present, amounts of manganese up to 4% may be added with very beneficial results as more fully hereinafter set forth. Iron and cobalt in amounts

5

10

15

20

25

30

35

40

45

50

55

of from 0.3 to 2.0% may also form useful but not absolutely necessary additions. I have also found that the properties of the alloys of this class as regards their ability to be worked by cutting or machining may be further improved by adding up to about 3% of lead.

As above indicated, I have found that it is desirable to add both manganese and aluminum for some purposes. This is recommended where increased strength and forgeability are desired.

10 Preferably, aluminum and manganese should be added in about the relative proportions of one part of aluminum to two parts of manganese, since it appears that the improved properties imparted by the presence of aluminum and manganese are due to the formation of a hard compound, probably MnAl, which gives increased strength to the matrix.

15 These alloys can be used as cast or be hot worked by forging, rolling, or especially, by extrusion; but to improve their structural properties for use in forming bearings and for similar purposes it is advisable to subject them to heat treatment.

20 According to a preferred form of heat treatment, the cast or hot worked piece is heated up to or above a point where the alloy forms a homogeneous beta phase or a mixture of the two betas possible—650°–800° C., according to the composition,—and then quenched or air cooled. This

25 brings it into a hard martensitoidal or acicular form. It is next heated to a point above the eutectoidal point, or from 550°–625° C., and kept at this temperature for from one to six hours, or until the acicular structure is destroyed and the beta phase divorces from the alpha, the first coalescing in the form of well-rounded dense grainlets sufficiently well spaced within the matrix of alpha to permit the formation of a lubricating 30 film on the surface when in use.

35 The next step consists in lowering the temperature preferably to 450°–525° C., and not below 250° C., and holding such temperature for such time as to allow the beta phase to dissociate into alpha plus delta, the latter forming very fine particles within each original grainlet of beta. When 40 this condition is reached the structure will have become stabilized.

45 When the alloy contains amounts of manganese and aluminum within the range hereinbefore indicated, the heat treatment may be still further modified. According to this further modification, the cast or hot worked piece is heated as in

5 the first instance above mentioned to above the range 650°–850° C., according to the composition, and preferably to or above 750° C., and then quickly cooled as by quenching or air cooling. The product so treated is then reheated to within the range 250°–525° C. and held for approximately one hour or until the delta constituent precipitates and becomes stabilized, whereupon it may be permitted to cool either slowly or rapidly.

10 What I claim is:

15 1. A composition of matter consisting principally of copper and containing 4–18% tin, 10–35% zinc, a substantial and effective amount but not exceeding 10% of nickel, and being substantially free from carbon; said composition being capable when subjected to heat treatment of assuming a physical structure characterized by the presence of beta crystals substantially uniformly distributed throughout a matrix of alpha crystals.

20 2. A composition of matter consisting principally of copper and containing 4–18% tin, 10–35% zinc and about 2–3% of nickel, and being substantially free from carbon; said composition being capable when subjected to heat treatment 25 of assuming a physical structure characterized by the presence of beta crystals substantially uniformly distributed throughout a matrix of alpha crystals.

25 3. A bronze alloy consisting of 4–18% tin, 30 10–35% zinc, about 2–3% nickel, substantial and effective amounts of aluminum and manganese, but not exceeding 2% aluminum and 4% manganese, with the balance principally copper, and being substantially free from carbon; said alloy 35 being capable when subjected to heat treatment of assuming a physical structure characterized by the presence of beta crystals substantially uniformly distributed throughout a matrix of alpha crystals.

40 4. A bronze alloy consisting of 4–18% tin, 10–35% zinc, substantial and effective amounts of nickel, aluminum, manganese and lead, but not exceeding 10% nickel, 2% aluminum, 4% manganese and 3% lead, with the balance principally copper, and being substantially free from carbon; said alloy being capable when subjected to heat treatment of assuming a physical structure characterized by the presence of beta crystals substantially uniformly distributed throughout a matrix of alpha crystals.

45 MICHAEL GEORGE CORSON.